

## UNITED STATES PATENT OFFICE.

MORTON ROLAND SHERBINO, OF DETROIT, MICHIGAN, ASSIGNOR TO HYDRAULIC BRAKE COMPANY, OF DETROIT, MICHIGAN, A CORPORATION OF CALIFORNIA.

## NONCORROSIIVE LIQUID FOR FLUID SYSTEMS.

\* No Drawing.

Application filed March 19, 1926. Serial No. 96,085.

This invention concerns rendering the corrosive fatty acids present in castor oil harmless to copper by saponifying the fatty acids, leaving the resulting soap in solution. Heretofore, it has been common practice to use a solution of alcohol and castor oil in substantially equal proportions as the actuating fluid medium of so-called hydraulic braking systems. This solution has been used because of the fact that castor oil thus dissolved in alcohol has no detrimental effect upon the rubber used for cup washers and for piping, and that at the temperatures encountered in practice, has a sufficiently constant viscosity for practical purposes. It has been found in practice that even chemically pure castor oil, when mixed with any commerical alcohols, brings about a gradual corrosion of copper, causing the copper to eventually dissolve in the castor oil.

I have found that the corrosion of the copper is greatly decreased by the saponification of the fatty acid present in the castor oil. By employing an alkali soluble in alcohol, such as sodium or potassium hydroxide, and adding the required amount (determined by the quantity of fatty acid present) to such an alcohol and castor oil solution as above described, there results an alcohol and castor oil solution of substantially equal proportions which is sufficiently free from fatty acids as to preclude any attack on copper metal used in the braking systems.

The amount of alkali necessary to bring about the saponification of the fatty acid can be roughly calculated by multiplying the percentage of fatty acid by eight, which gives the grams of alkali necessary per gallon of castor oil.

I prefer to use potassium hydroxide (KOH), as the resulting soap, being a liquid, is much less affected by cold tempera-

tures than the soap resulting from saponification with sodium hydroxide.

I claim:

1. As the liquid medium of a fluid system, a solution of castor oil and alcohol rendered non-corrosive to copper by the saponification of the fatty acid.

2. A solution of castor oil and alcohol rendered non-corrosive to copper by the saponification of the fatty acid with the resulting soap left in solution as an inert substance.

3. The method of rendering a solution of castor oil and alcohol non-corrosive to copper which consists in saponifying the fatty acid.

4. The method of minimizing the corrosive effect of a castor oil and alcohol solution upon copper which consists in saponifying the fatty acid of the oil and leaving the saponification products thereof in the solution.

5. A liquid medium of a fluid system exposed to copper, which comprises a solution of alcohol and an oil soluble therein and a product held in the solution and formed by the saponification of the fatty acid of the castor oil.

6. A liquid medium for a fluid system exposed to copper which comprises a solution of alcohol and castor oil containing a small quantity of potassium hydroxide for the purpose specified.

7. In a fluid brake system, the combination with a liquid medium, comprising castor oil, in contact with metallic copper of means carried in the medium for minimizing the destructive action of the fatty acid of the oil upon the copper, said means comprising an alkali for saponifying the fatty acid.

In witness whereof, I hereunto subscribe my name this 2nd day of March, 1926.

MORTON ROLAND SHERBINO.